

No. 813,123.

PATENTED FEB. 20, 1906.

J. TRUE.

METHOD OF MAKING GLASS ORNAMENTS.

APPLICATION FILED SEPT. 12, 1905.

FIG. 1.



FIG. 2.



FIG. 3.



FIG. 4.



FIG. 5.



Witnesses

J. True  
L. H. Schmidt.

Inventor  
Jacob True,

By *Malvinae* *Malvinae*  
Attorneys.

# UNITED STATES PATENT OFFICE.

JACOB TRUE, OF CASTILE, NEW YORK.

## METHOD OF MAKING GLASS ORNAMENTS.

No. 813,123.

Specification of Letters Patent.

Patented Feb. 20, 1906.

Application filed September 12, 1905. Serial No. 278,115.

*To all whom it may concern:*

Be it known that I, JACOB TRUE, a citizen of the United States, residing at Castile, in the county of Wyoming and State of New

5 York, have invented certain new and useful Improvements in Methods of Making Glass Ornaments, of which the following is a specification.

10 The object of my invention is to provide an improved method of making glass ornaments.

For a full description of the invention and the manner in which it is carried out reference is to be had to the accompanying drawings, in which—

15 Figures 1 to 5, inclusive, represent some of the different ornamental articles which may be produced by my improved method, the shading on said figures representing the peculiar finished surface of the glass that my 20 method provides.

In carrying out the improved method I first take a piece of glass of the approximate size of the article I desire to produce, but somewhat larger than the same, and preferably 25 lay it upon a cushion or several layers of felt or some other similar soft article to take up the shock of the subsequent operation or steps and then by striking or hammering on the edge of the glass I chip off therefrom 30 around the margin small particles of the glass according to the finished outline which I desire to produce until the glass has assumed substantially the desired margin, contour, or configuration. At those points where 35 the outline has not been rendered sufficiently distinct by means of the hammering or striking operation I finish the same by the use of a file, which I preferably first dip in water or milk, using the edge of the file against the 40 margin of the glass to form notches or the like, as may be desired, for the finishing operation. If desired, I may use the same file for the hammering and striking operation, as de-

scribed, and having become expert in my method I may hold the glass in my hand 45 while operating upon it instead of laying it upon a cushion or similar soft surface.

It is to be particularly noted that in addition to the novelty itself, which resides in first hammering against the margin of the 50 glass to produce the desired contour and then subsequently filing any slightly-irregular points or places which may have remained, my invention produces by the chipping or hammering process a peculiar flaky 55 border around the finished article as designated by the shading in the various figures of the drawings, and this flaky margin adds greatly to the appearance of the ornamental article, as it provides innumerable angles 60 and surfaces for the reflection of the light, causing the article to possess irradiating characteristics.

It is evident as described by the foregoing and illustrated in the drawings that my invention is capable of producing ornamental 65 glass articles of various shapes or designs.

Having thus described the invention, what is claimed as new is—

The herein-described improved method of 70 making glass ornaments with marginal edges provided with innumerable angles to impart to the ornament an iridescent appearance at the edges, consisting of striking the pieces of glass with a file to produce the desired outline in the rough and subsequently filing the 75 edges to form notches for completing the operation, the file being first dipped in water or milk.

In testimony whereof I affix my signature 80 in presence of two witnesses.

JACOB TRUE. [L. s.]

Witnesses:

MARCUS E. POND,  
ANDREW L. JOHNSON.